

## UNITED STATES PATENT OFFICE

2,024,545

## DENTAL ALLOY

James R. Stack, Milford, Del., assignor to The  
L. D. Caulk Company, Milford, Del., a corpora-  
tion of Delaware

No Drawing. Application October 4, 1933,  
Serial No. 692,129

3 Claims. (CL 75—1)

This invention relates to dental alloys and particularly to silver-tin dental alloys containing beryllium.

It has been found that by incorporating relatively small and definite quantities of beryllium in silver-tin base dental alloys, the resulting alloy will, upon amalgamation with mercury, exhibit many desirable and beneficial properties. For example, the presence of proper amounts of beryllium in the alloy in addition to increasing the hardness of both the alloy and the amalgam made therefrom imparts a perceptibly higher crushing strength to the latter.

Among other features of the invention, is the ability of the amalgam to resist tarnishing and retard corrosion after insertion in the cavity of the tooth.

In preparing the improved silver-tin base alloys of the present invention, the constituents may be placed in a suitable furnace and melted under cover of a non-oxidizing atmosphere. Sufficient beryllium is incorporated in the melt to yield the desired percentage in the finished alloy. The alloy may then be cast, milled to the correct particle size and annealed.

As regards the amount of beryllium incorporated in the alloy, it has been found that the quantity should be sufficient to constitute not less than 0.06% nor more than 1.0% of the final alloy. In other words, at least 0.06% of beryllium is necessary to impart the desirable properties to the alloy to an appreciable degree, while if more than 1.0% of beryllium is used the beneficial effects tend to disappear or are completely nullified. For most silver-tin base dental alloys, a beryllium content lying between the limits of 0.1% to 0.6% appears to give the most satisfactory results.

It may be preferable from an operating standpoint to add the beryllium in some other form than as elemental beryllium. For example, in manufacturing a silver-tin base dental alloy having an appreciable copper content, the beryllium may be added in the form of a beryllium-copper alloy comprising, for example, 12½% beryllium. Again, the alloy may be made by blending a dental alloy containing more than

the desired amount of beryllium with a similar dental alloy containing no beryllium. In any event, however, the final product should contain not less than 0.06% or more than 1.0% of beryllium and preferably only 0.1% to 0.6% of that element.

While the invention is applicable to all silver-tin dental alloys, the alloy preferably should conform to the following well recognized specification:

|        |             |
|--------|-------------|
| Silver | 65% minimum |
| Tin    | 25% minimum |
| Copper | 6% maximum  |
| Zinc   | 2% maximum  |

In addition to the characteristics heretofore mentioned, it has also been found that the presence of beryllium within the limits specified decreases the setting time of amalgams formed from the alloy. This characteristic is desirable in some instances. However, the setting time may, if desired, be increased by annealing the alloy at higher temperatures, for example 500° F. or more, than are usually employed in annealing ordinary silver-tin base dental alloys.

While certain novel features of the invention have been disclosed and are pointed out in the annexed claims, it will be understood that various omissions, substitutions and changes may be made by those skilled in the art without departing from the spirit of the invention.

What is claimed is:

1. A silver-tin base dental alloy containing a minimum of 65% silver, a minimum of 25% tin and from 0.06% to 1.0% beryllium, which upon amalgamation with mercury exhibits improved hardness and marked resistance to corrosion.

2. A silver-tin base dental alloy containing a minimum of 65% silver, a minimum of 25% tin and from 0.1% to 0.6% beryllium, which upon amalgamation with mercury exhibits improved hardness and marked resistance to corrosion.

3. A dental alloy consisting of a minimum of 65% silver, a minimum of 25% tin, copper not exceeding 6%, zinc not exceeding 2%, and from 0.06% to 1% beryllium.

JAMES R. STACK.